

# UNITED STATES PATENT OFFICE.

PATRICK H. DEAN, OF WINCHESTER, INDIANA.

## IMPROVEMENT IN PHOTOGRAPHIC VARNISHES.

Specification forming part of Letters Patent No. **149,449**, dated April 7, 1874; application filed February 25, 1874.

*To all whom it may concern:*

Be it known that I, PATRICK H. DEAN, of Winchester, in the county of Randolph and State of Indiana, have invented a certain Improved Compound for Varnishing Photographs, of which the following is a specification:

This invention relates to that class of compounds used for varnishing or enameling photographs; and it consists of a composition formed by mixing castile-soap and glycerine with alcohol and liquid ammonia.

To prepare the varnish, take twenty-four (24) grains of castile-soap, one-quarter ( $\frac{1}{4}$ ) of an ounce of glycerine, six (6) ounces of alcohol, and one-half ( $\frac{1}{2}$ ) of an ounce of liquid ammonia. These ingredients are thoroughly mixed together, and heated in a suitable vessel to effect their intimate union.

The varnish thus prepared is applied in a liquid state to the face of a photograph by means of a swab or brush, and after it has become dry, the photograph is subjected to the action of a heated burnisher or like instru-

ment, as usual. By this means the thin coat of varnish is excited, and, together with the albumen on the paper, gives a permanent gloss or polish to the photograph.

I have found by actual tests that the varnish above described is superior to any now in most general use, and doubt not that it will be generally adopted by the profession when once known.

What I claim as my invention, and desire to secure by Letters Patent, is—

The herein-described compound for varnishing photographs, consisting of a mixture of castile-soap, glycerine, alcohol, and liquid ammonia, in about the proportions and prepared substantially in the manner specified.

In testimony whereof I have signed my name to this specification in the presence of two subscribing witnesses.

PATRICK H. DEAN.

Witnesses:

C. S. KELLEY,  
JNO. E. NEFF.